

# United States Patent Office

2,929,676

Patented Mar. 22, 1960

1

2,929,676

## PRODUCTION OF ALKALI METAL BOROHYDRIDES

William H. Schechter, Zelienople, Pa., assignor to Callery Chemical Company, Pittsburgh, Pa., a corporation of Pennsylvania

No Drawing. Original application March 17, 1953, Serial No. 342,993. Divided and this application November 21, 1956, Serial No. 623,539

4 Claims. (Cl. 23—14)

This invention relates to the production of alkali metal borohydrides,  $MBH_4$ , in which M is an alkali metal, and more particularly to their production by the reaction of an alkali metal, hydrogen, and an alkali metal fluoborate,  $MBF_4$ .

The metallic borohydrides are excellent reducing agents, they provide efficient sources of hydrogen, and they may be used for the production of various boron compounds, e.g., diborane and related boranes, which in turn are desired for certain purposes, e.g., for thermal conversion to other boron hydrides. The methods known for the production of boranes and metallic borohydrides are characterized by low yields or they require highly skilled operating technique. Generally speaking, they are adapted only to batch operation, and the products made by procedures known heretofore are consequently quite expensive.

The primary object of the invention is to provide a simple and easily performed method for the making of alkali metal borohydrides which is simple and efficient, may be practiced with readily available inexpensive starting materials, is not dependent upon highly skilled operating technique, and is more direct and more easily practiced to provide these products at less expense than is the case with previously known methods.

A further object is to provide a method embodying the foregoing object which is adapted to continuous operation.

Another object is to provide metallic borohydrides in a form exhibiting low bulk density and of exceptionally high activity.

A further object is to provide sodium borohydride in accordance with the foregoing objects.

Other objects will be recognized from the following specification.

This invention is based on the discovery that a finely divided alkali metal, hydrogen, and an alkali metal fluoborate react at elevated temperatures according to the equation  $4M + 2H_2 + MBF_4 = MBH_4 + 4MF$  to produce an alkali metal borohydride. The reaction is performed in a closed system and under anhydrous conditions. Alkali metals, such as sodium, potassium or lithium, or mixtures of alkali metals with one another such as sodium-potassium alloy, or with other metals may be used. Also, any alkali metal fluoborates, such as lithium, sodium or potassium fluoborate may be used in the foregoing reaction with corresponding production of alkali metal borohydride.

In the preferred embodiment of the invention the alkali metal is dispersed in an inert liquid. The alkali metal is dispersed as finely as possible in the heated inert liquid, most suitably one of high boiling point such as mineral oil. Other appropriate inert liquids are, of course, available and will occur to workers in the field. Hydrogen and the alkali metal fluoborate are then introduced into the heated alkali metal suspension, or dispersion, while agitating or stirring it violently. If preferred, the alkali metal fluoborate may be introduced along with the alkali

2

metal. Maintenance of fine dispersion during the reaction is, I find, essential. This may be accomplished suitably by the use of a high speed stirrer, such as a flat bladed turbine or a slotted impellor of the type known as a "Dispersato r." Hydrogen may be provided for reaction simply by maintaining a hydrogen atmosphere over the agitated dispersion, or it may be injected into the agitated dispersion, or it may be injected through the agitator bearing unit so as to be expelled through perforations in the stirrer blades. It is preferred to use baffled containers in accordance with modern mixing practices.

In the production of alkali metal borohydrides according to the foregoing reaction the alkali metal, and the alkali metal fluoborate, finely dispersed or suspended in an inert liquid is heated to  $250^\circ$  to  $265^\circ$ , or higher, e.g.  $320^\circ$  C., and while agitating violently, dry hydrogen is introduced into this suspension. When reaction has been completed the reaction body is cooled and filtered, and the solid residue is washed with solvent for the suspension liquid, e.g. petroleum ether in the case of mineral oil. The borohydride is then extracted from the alkali metal halides, as by liquid ammonia at  $-33^\circ$  C. and the borohydride then recovered by evaporation of the ammonia. Other selective solvents for the borohydride, such as amines and polyethylenedialkylethers, may also be used.

Following this procedure sodium borohydride of as high as 80 to 94% purity has been made using sodium fluoborate and sodium as the alkali metal from reactions of 4 hours duration at  $280^\circ$  C.

At temperatures below  $250^\circ$  C., e.g.  $220^\circ$  C., the reaction is so slow as to be impractical. It has been found that at higher temperatures, i.e. at about  $320^\circ$ , that secondary reactions of an undetermined character decrease the yield of borohydride. A reaction of 3 hours duration at  $275^\circ$  C. gave a 75% yield of sodium borohydride, while a reaction of 3 hours duration at  $320^\circ$  C., resulted in a yield of only 27%. Although the desired reaction proceeds to some extent at higher temperatures, i.e.  $350^\circ$  C., it is preferred to operate at temperatures below  $320^\circ$  C.

The reaction is exothermic, and the inert liquid functions as a heat sink and increases the rate at which heat can be transferred to and from the reaction, thus facilitating the temperature control of the reaction.

In the practice just described the practice may be operated at or slightly above atmospheric pressure. I find, however, that it is advantageous to operate in an autoclave under superatmospheric, e.g. at 100 or 150 p.s.i.g., as at elevated hydrogen pressures the rate at which the reaction proceeds is increased.

The reaction may be aided, if desired, by having present in the suspension a small amount of stearic acid as a catalyst.

This application is a division of my copending application, Serial Number 342,993, filed March 17, 1953, which is a continuation-in-part of my application, Ser. No. 229,142, filed May 31, 1951, both now abandoned.

According to the provisions of the patent statutes, I have explained the principle and mode of practicing my invention and have described what I now consider to represent its best embodiment. However, I desire to have it understood, that within the scope of the appended claims, the invention may be practiced otherwise than as specifically, described.

I claim:

1. A method of making an alkali metal borohydride comprising dispersing an alkali metal in an inert liquid at a temperature of about  $250^\circ$  to  $350^\circ$  C., and introducing dry hydrogen and an alkali metal fluoborate into the dispersion, and thereby producing said borohydride, and recovering said borohydride from the system.
2. A method according to claim 1 in which the alkali

metal is sodium, the alkali metal fluoborate is sodium fluoborate and the borohydride recovered is sodium borohydride.

3. A method according to claim 2 in which the inert liquid is mineral oil.

4. A method according to claim 3 in which the pressure is between atmospheric and 150 p.s.i.

## References Cited in the file of this patent

## UNITED STATES PATENTS

|             |            |               |
|-------------|------------|---------------|
| 2,469,879   | Hurd       | May 10, 1949  |
| 5 2,532,217 | Winternitz | Nov. 28, 1950 |
| 2,720,444   | Banus      | Oct. 11, 1955 |
| 2,741,539   | Banus      | Apr. 10, 1956 |